

## UNITED STATES PATENT OFFICE

OTTO MATTHIES AND BRUNO WENDT, OF DESSAU IN ANHALT, GERMANY, ASSIGNEES  
TO AGFA ANSCO CORPORATION, OF BINGHAMTON, NEW YORK, A CORPORATION OF  
NEW YORK

LIGHT-SENSITIVE SILVER-HALIDE EMULSIONS AND PROCESS OF MANUFACTURING  
THE SAME

No Drawing. Application filed January 28, 1929, Serial No. 335,732, and in Germany January 31, 1928.

The present invention relates to photographic silver salt emulsions of increased stability, little tendency to fog and determined grain size, to layers containing the same and to a process for manufacturing the same.

In our co-pending application Ser. No. 335,733, filed this same day we have stated that compounds with three or more nitrogen compounds in the molecule one of which is linked to hydrogen being liable to substitution by silver and forming stable silver salts of no higher solubility than silver chloride are good stabilizers for photographic emulsions.

15 We found that also sulphur compounds forming stable silver salts with the group — $\text{S}\text{Ag}$ , these silver salts having the solubility characteristics cited above, can be employed for the same purpose in emulsion manufacture. They may be added to the finished emulsion or to its constituents at any stage of their manufacture or of emulsion-making. The compounds which form silver salts of the least solubility exert the strongest effect on 25 the stability of emulsions.

We further found that the said compounds when present during the addition of the silver nitrate solution restrain the growing of silver bromide grains and thus give to the emulsion 30 a steeper gradation while at the same time increasing its stability.

By our present process we may thus obtain emulsions of varying steepness of gradation though starting with the same proportions of 35 constituents.

The following examples illustrate the invention:

Example 1.—A highly sensitive negative emulsion is made according to any known 40 prescription and before the silver solution is run into the potassium bromide solution there are added to the latter 100 milligrams of thioglycollic acid per each 100 grams of silver nitrate. There is thus obtained a very finely 45 grained, hard emulsion, which is particularly suitable for copying black and white work.

Example 2.—The procedure is the same as that described in Example 1, using as the 50 added substance 50 milligrams of thiolactic acid. There is obtained an emulsion which

is suitable as a cinema film positive-emulsion.

Example 3.—To a negative emulsion made with a gelatine which produces fog according to any known prescription, there are added per kilo of emulsion, before the pouring operation, 7 milligrams of 2,6-dimercapto-4-keto-3,5-diphenylpenthiophen. There is obtained an improvement in durability amounting to 50 per cent. 55

Example 4.—There are added to a positive-emulsion, made as described in Example 2 or by any other process, before the pouring operation, 20 milligrams of allylaminothiobiazolesulphhydrate per kilo of emulsion. There is obtained an improvement of durability amounting to 100 per cent. 60

We claim:

1. A process of manufacturing light sensitive silver halide emulsions of increased stability, in which there is added to the emulsion a sulphur compound forming a stable silver salt with the group — $\text{S}\text{Ag}$  and having no higher solubility than silver chloride. 70

2. A process of manufacturing light sensitive silver halide emulsions of increased stability, in which there is added to a constituent of the emulsion at any stage of the manufacture a sulphur compound forming a stable silver salt with the group — $\text{S}\text{Ag}$  and having no higher solubility than silver chloride. 75

3. A process of manufacturing light sensitive silver halide emulsions of increased stability and restrained size of silver halide grains, in which there is added to a constituent of the emulsion prior to the addition of silver nitrate a sulphur compound forming a stable silver salt with the group — $\text{S}\text{Ag}$  and having no higher solubility than silver chloride. 80

4. A process of manufacturing light sensitive silver halide emulsions comprising the step of adding allylaminothiobiazolesulphhydrate. 90

5. A process of manufacturing light sensitive silver halide emulsions comprising the step of adding allylaminothiobiazolesulphhydrate to a constituent of the emulsion at any stage of its manufacture. 95

6. Light sensitive silver halide emulsions containing a sulphur compound forming a 100

stable silver salt with the group — $\text{S}\text{Ag}$  and having no higher solubility than silver chloride.

7. Light sensitive silver halide emulsions containing allylaminothiobiazolesulfhydrates.

8. In testimony whereof, we affix our signatures.

OTTO MATTHIES.  
BRUNO WENDT.

10

15

20

25

30

35

40

45

50

55

60

65